

## UNITED STATES PATENT OFFICE

2,089,191

## PRODUCTION OF TEXTILE THREADS AND FABRICS

Henry Dreyfus, London, and Donald Finlayson, Spondon, near Derby, England, assignors to Celanese Corporation of America, a corporation of Delaware

No Drawing. Application January 30, 1935, Serial No. 4,085. In Great Britain February 9, 1934

10 Claims. (Cl. 117—2)

This invention relates to the manufacture of crêpe threads of cellulose acetate or other cellulose ester or ether and to the production of fabrics therefrom.

5 It is well known that valuable fabrics may be produced with the aid of natural silk yarns which have been highly twisted while in the gummed state. After an aqueous scouring treatment such fabrics exhibit the well known crêpe effects and 10 are highly valued on account of their pleasing appearance and handle. The production of crêpe fabrics in an analogous manner by the use of highly twisted cellulose acetate threads is, however, accompanied by great difficulties. Generally, the crêpe effect obtained by simply applying to a cellulose acetate thread a twist of the order of that commonly employed in connection with natural silk, weaving the twisted threads into a fabric and scouring the latter, 15 is very unsubstantial and not comparable with that obtained with natural silk or regenerated cellulose artificial silk.

It has now been found that by crêpe twisting threads of cellulose acetate or other cellulose esters or ethers in the presence of hot water, it is possible to produce cellulose acetate or other cellulose ester or ether crêpe threads having, as compared with threads produced by a simple twisting operation, greatly improved properties, particularly as regards strength and the ability 20 to yield fabrics exhibiting good crêpe effects.

In accordance with the present invention, therefore, in the production of highly twisted crêpe threads of cellulose acetate or other cellulose ester or ether, the threads are treated with hot water at atmospheric pressure or at any desired pressure during the actual application of crêpe twist. Thus, the twisting operation may be conducted so that at least a portion of that 25 part of the track of the running thread in which twisting actually takes place, lies through a body of hot water. For example, the thread may be twisted on a device of the kind in which the thread is drawn off over the end of a rotating package and allowed to pass through hot water on its way to a winding device.

The invention is of particular importance in connection with the production of cellulose acetate crêpe threads and will be more particularly 30 described with reference to the production of such threads.

The threads may consist of substantially continuous filaments of cellulose acetate or they may consist of discontinuous filaments, the length 35 of which may vary within wide limits. For ex-

ample the threads may be those spun from a mass of discontinuous filaments or those prepared in the manner described in British Patents Nos. 424,683, 424,752, 424,830 and 424,875.

If desired the filaments of the threads may contain water-insoluble compounds, whether compounds of pigment-like character in such form as materially to modify the lustre of the filaments (e. g. barium sulphate or titanium dioxide), or loading metal compounds, for example tin compounds.

In carrying out the new process twisting is most advantageously effected on a device of the kind in which the thread is drawn off over the end of a rotating package through a guide fixed substantially in line with the axis of rotation of the package and is thereafter wound on a bobbin or the like, the thread being passed through hot water on its way from the guide to the bobbin. In this way the yarn is subjected to the action of the hot water during the actual application of twist.

On the other hand, any other suitable crêpe twisting device may be employed. For example a ring twister may be used for the crêpe twisting of thread consisting of discontinuous cellulose acetate filaments. An essential characteristic of a ring twisting device is that the thread is twisted as it is wound on to a rotating package.

The twisting spindle, the guide fixed in line with the axis of the spindle, and the hot water treatment device, should be so arranged that the twist resulting from the rotation of the package is at least partly inserted while the thread is in contact with hot water. If the freedom of the thread to rotate within the balloon guide or other guide preceding or forming part of the hot water treatment device is unduly restricted, e. g. by causing the thread to change direction materially at the guides, the insertion of twist while the thread is in contact with hot water may be restricted to an undesirable extent or substantially prevented and the resulting crêpe threads may not have the valuable properties which may otherwise be secured. Using a twisting device of the kind in which thread is drawn off over the end of a rotating package, it is advantageous to arrange that the path of the thread after leaving the balloon guide and through the hot water treatment device, is substantially in line with the axis of the spindle.

If desired, the above-mentioned twisting devices, in which the thread is drawn off over the end of a rotating package, may be provided with

a device which restricts the ballooning of the thread or the tendency of twist to run back to the package. As examples of such devices may be mentioned flyers and the floating ring device described in U. S. Patent No. 1,784,581. The latter device is of particular value when the thread to be twisted is of very low twist, for example less than about 1 turn per inch.

The treatment of the thread with hot water during twisting may be effected by drawing the thread off from a twisting spindle and passing it upwardly through a small hole in a suitable receptacle containing hot water, the thread then passing to a winding device. The hole may be, for example, about  $\frac{1}{2}$  of an inch in diameter and may be provided with means adapted to lead away and prevent from reaching the twisting spindle, any liquid issuing from the hole. If desired, the hole may take the form of a short tube of fine bore, fixed in the receptacle, whereby the flow of liquid from the receptacle at the point of entrance of the thread may be reduced. Another method is to supply hot water to the thread. For example, the thread may be caused to pass in contact with a horizontally disposed roller, preferably circumferentially grooved, arranged to rotate in a bath of hot water and so to carry water to the thread.

The duration of the treatment with hot water may be relatively short, such as may be secured when the thread is travelling at a speed of 2-10 metres per minute and is in contact with hot water for 1-3 inches of its travel. Lengthier treatments may however be employed.

Very good results may be obtained by using hot water at temperatures of 85-100° C. Preferably the water should be as hot as possible and temperatures of, for instance, 95-100° C. are to be recommended. If desired, the hot water may be employed under pressure, for example 2-10 or 15 pounds or more per square inch. The use of pressure enables the water to be employed at higher temperatures than is possible under atmospheric pressure. By using pressure, therefore, the temperature of the water may be above 100° C. and up to the boiling point of water at the pressure employed. Water may be employed under pressure, however, when the temperature is below 100° C.

The initial thread may already be twisted to a small degree, for example up to 10 turns per inch, e. g. to 2-5 turns per inch or to such small degree as is commonly applied in the production of cellulose acetate threads by dry spinning cellulose acetate solutions and winding and twisting the resultant filaments on a cap twisting device.

In carrying out the new process the crêpe twist may be applied in a single stage. If desired, however, the crêpe twist may be applied in two or more stages, the final stage of twisting being effected whilst treating the thread with hot water.

When the crêpe twist is applied in two or more stages the advantages of the process may be obtained when not only the final stage of the crêpe twisting but an earlier stage or stages of twisting are also effected while treating the thread with hot water. In fact it is of great advantage to effect while treating the thread with hot water, any application of twist beyond the point at which twisting would result in weakening of the thread if the said twisting were effected without the hot water treatment.

The precise degree of twist beyond which it is important to treat with hot water during twist-

ing depends upon the total denier of the thread and the number of its constituent filaments. Generally at least the last two thirds of the total crêpe twist should be applied whilst treating the thread with hot water.

The cellulose acetate filaments of the threads very readily undergo stretching when the threads are twisted during treatment with hot water. The amount of stretch may be measured by comparing the original thread denier with the final thread denier (after untwisting). The denier of the resultant thread is, in general, owing to imparted stretch, less and even substantially less than if the hot water treatment is omitted. The stretch imparted to the filaments of the threads during the twisting operation may for example be of the order of 5-30% of their original length, and particularly 10-20%. The degree of stretching of the filaments of the thread may be such that the final denier of the crêpe twisted thread is not much in excess of or is even the same or less than the denier of the thread prior to crêpe twisting. For example the stretch may be such that the denier of the crêpe twisted thread is from 95 to 115%, particularly 100 to 110% of that of the thread before crêpe twisting, especially in the case of threads having an original denier of 200 or less. Good crêpe fabrics may, however, be obtained when the final denier is still greater, for example up to 120% of that of the thread before twisting, particularly when still heavier threads are employed, i. e. threads having a denier above 200.

The total twist applied in accordance with the new process may vary within wide limits. The new process possesses the feature that it enables a very high degree of twist to be applied without the great weakening of the thread such as is generally experienced when a cellulose acetate thread is simply crêpe twisted. The process, moreover, permits the insertion of twists which are impossible of attainment without the hot water treatment owing to breakage of the thread. This is important since it enables crêpe fabrics to be produced having very pronounced crêpe effects. The crêpe figure can be regulated according to requirements. The total twist desirable in any particular case depends upon a number of factors, including the precise effects required, and the denier of the thread. For example, with threads of 150 denier twists of about 70 to 75 or more turns per inch are desirable, and with 100 denier threads twists of about 90 to 100 or more turns per inch. With these indications it is a simple matter to determine the desirable twists for threads of other deniers.

When the crêpe twist is applied in two or more stages the twist may be divided between the twisting stages in various proportions. Twist applied in the absence of the hot water treatment should not be of such degree as to damage the thread. To this end, as indicated previously, twisting without the hot water treatment should not be effected where the twist applied is sufficient to result in substantial weakening of the thread.

A particularly convenient method of working is to apply about one sixth to one quarter of the total crêpe twist without the hot water treatment, say up to 10 or 15-25 or even in some cases 70 to 30 turns per inch, and then to complete the crêpe twist while treating with hot water.

By the new process highly twisted cellulose acetate crêpe threads may be produced which are smooth and cylindrical and in which the fila-

ments are extremely closely packed. For example, threads may be obtained which have an apparent specific gravity, as determined from the diameter and denier, of more than 85 per cent., e. g. 85-90 per cent., of the actual specific gravity of the filaments. As appears from microscopic examination of the cross-sections of threads twisted in accordance with the invention, the filaments are squeezed together into 10 substantially as close contact as possible, causing some distortion of at least some of them. The filaments, however, are not stuck together and can be separated upon untwisting.

While the new process enables production of 15 threads which yield satisfactory crêpe effects without a special treatment, other than the twisting and hot water treatment characteristic of the process, other devices and treatments may, if desired, be employed further to improve the properties of the crêpe threads and/or fabrics produced therefrom. For example, the crêpe threads may be sized at any suitable stage of their manufacture, for example in the course of winding on to the bobbin from which twisting is 20 effected. In this connection, particular mention may be made of sizing materials selected in accordance with the considerations laid down in U. S. application S. No. 491,070 filed 24th October 1930 which has issued as Patent No. 30,007,182. For example a casein, egg-albumen, or other size which is not very readily removed by aqueous treatments may be employed. Another size which may be employed is a drying oil, if desired one which has been partially oxidized, e. g. 25 boiled or blown linseed oil.

The highly twisted crêpe threads may be incorporated in the fabrics in various ways, for example the weft alone may be wholly or partially composed of such threads or the warp may also 30 contain them. Valuable fabrics may be produced by employing warp threads of relatively low twist and in the weft both crêpe threads having a left-hand twist and crêpe threads having a right-hand twist, pairs of threads of left-hand twist alternating with pairs of threads of right-hand twist.

If desired the cellulose acetate crêpe threads may be associated in the fabrics with highly twisted crêpe threads of other materials, e. g. of 40 natural silk or regenerated cellulose, or with highly twisted threads produced by other processes. Where the fabrics contain threads of low twist these may be wholly of cellulose acetate or wholly or in part of other materials, e. g. natural 45 silk or regenerated cellulose.

Fabrics containing highly twisted crêpe threads prepared in accordance with the invention may be subjected to a hot aqueous treatment in the manner commonly adopted in connection with 50 fabrics comprising highly twisted yarns of natural silk. The delustring effect of hot aqueous baths upon fabrics containing threads of lustrous cellulose acetate may be minimized by incorporation therein of salts or sugars.

Crêpe threads of organic esters of cellulose other than cellulose acetate, or of cellulose ethers, and fabrics containing such threads may be prepared in a manner similar to that described in the case of cellulose acetate threads. As examples of 60 such other cellulose esters or ethers may be mentioned cellulose formate, propionate or butyrate, and methyl, ethyl, or benzyl cellulose. Organic esters of cellulose and cellulose ethers, are referred to in the appended claims as "organic derivatives of cellulose".

What we claim and desire to secure by Letters Patent is:—

1. Process for the production of a highly twisted crepe thread of filaments of an organic derivative of cellulose, which comprises crepe twisting a 5 thread of filaments of an organic derivative of cellulose, the thread of filaments being subjected to the action of hot water during the actual insertion of at least the last part of the crepe twist.

2. Process for the production of a highly twisted 10 crepe thread of filaments of an organic derivative of cellulose, which comprises crepe twisting a thread of filaments of an organic derivative of cellulose, and during at least the last part of the twisting passing the thread through water at a 15 temperature above 95° C. so that the thread of filaments is wetted with the hot water during the actual insertion of at least the last part of the crepe twist.

3. Process for the production of a highly twisted 20 crepe thread of cellulose acetate filaments, which comprises crepe twisting a thread of cellulose acetate filaments, the thread of filaments being subjected to the action of hot water during the actual insertion of at least the last part of the 25 crepe twist.

4. Process for the production of a highly twisted crepe thread of cellulose acetate filaments, which comprises crepe twisting a thread of cellulose acetate filaments, and during at least the last 30 part of the twisting passing the thread through water at a temperature above 95° C. so that the thread of filaments is wetted with the hot water during the actual insertion of at least the last part of the crepe twist.

5. Process for the production of a highly twisted crepe thread of cellulose acetate filaments, which comprises crepe twisting a thread of cellulose acetate filaments in a single stage, the thread of filaments being wetted with hot water during the 40 actual insertion of the crepe twist.

6. Process for the production of a highly twisted crepe thread of cellulose acetate filaments, which comprises crepe twisting a thread of cellulose acetate filaments in at least two stages, of which 45 the final stage involves insertion of from two-thirds to five-sixths of the total twist, and wetting the thread of filaments with hot water during the actual insertion of the twist in the final stage.

7. Process for the production of a highly twisted 50 crepe thread of cellulose acetate filaments, which comprises crepe twisting a thread of cellulose acetate filaments, the thread of filaments being wetted with hot water during the actual insertion of at least the last part of the crepe twist, and the filaments of the thread being stretched so that the denier of the crepe twisted thread is 95 to 115% of that of the thread before crepe twisting.

8. Process for the production of a highly twisted 60 crepe thread of cellulose acetate filaments, which comprises crepe twisting a thread of cellulose acetate filaments, and during at least the last part of the twisting passing the thread through hot water in a container having below the water level 65 a small hole for the passage of the thread, so that the thread of filaments is wetted with the hot water during the actual insertion of at least the last part of the crepe twist, at least the last part of the twisting being effected by the rotation of a package from which the thread is being drawn.

9. Process for the production of a highly twisted crepe thread of cellulose acetate filaments, which comprises crepe twisting a thread of cellulose acetate filaments, and during at least the last 70 75

part of the twisting passing the thread through hot water so that the thread of filaments is wetted with the hot water during the actual insertion of at least the last part of the crepe twist, at least the last part of the twisting being effected by rotation of a package on which the thread is being wound.

5 10. Process for the production of a crepe fabric, which comprises crepe twisting a thread of cellu-

lose acetate filaments, the thread of filaments being wetted with hot water during the actual insertion of at least the last part of the crepe twist, incorporating the crepe twisted thread in a fabric, and thereafter subjecting the fabric to 5 a hot aqueous treatment.

HENRY DREYFUS.  
DONALD FINLAYSON.